

UNITED STATES PATENT OFFICE

JEAN GEORGES KERN, OF WALTHAM, MASSACHUSETTS, AND CHARLES J. SALA, OF  
WILMINGTON, DELAWARE, ASSIGNORS TO E. I. DU PONT DE NEMOURS & COMPANY,  
OF WILMINGTON, DELAWARE, A CORPORATION OF DELAWARE

## PRINTING PASTE

No Drawing. Original application filed August 4, 1927, Serial No. 210,714. Divided and this application filed March 21, 1930. Serial No. 437,941.

This case is a division of our copending application Serial No. 210,714, filed August 4, 1927.

it is found that an excess of base is necessary to give the most satisfactory results.

When preparing the products obtained from the sulfonated fatty acids we may proceed as follows:

This invention relates to alkylolamine salts of aliphatic acids both saturated and unsaturated and to the sulfonic acid derivatives of these acids and more particularly to the ethanolamine salts of the higher fatty acids.

The acid product of the mixture of the sulfonated unsaturated acid as obtained by the action of sulfuric acid on an unsaturated oil such as castor oil in the well known man-

This invention has as objects the preparation of soluble oils, solvents and detergents as well as of antiseptic soaps.

on such as castor oil in the well known manner is freed of mineral acid by washing. It is then freed of water either by settling or by

These objects are accomplished by making the salts of the bases known as alkylolamines or hydroxy-alkylamines, more particularly of the ethanolamines, by combination with the fatty acids mentioned above by any of the well known methods for the production of salts.

any other suitable means and then enough of the alkylolamine base is added at ordinary temperature to neutralize the acidity of the sulfonic acid group or of both sulfonic acid and the carboxylic acid groups. The following examples will serve to illustrate our method of procedure, but it is to be under-

The bases used for our purpose may be represented by the following general formula:

stood that the invention is not to be limited thereby:



25 where Alk represents an aliphatic or hydroxy aliphatic radical,  $R_1$  and  $R_2$  represent hydrogen or an aliphatic radical or a hydroxy aliphatic radical or a poly hydroxy aliphatic radical. In making these new soluble oils we  
30 may proceed as follows:

1960 parts of oleic acid are mixed with  
950 parts of a mixture containing 75% tri-ethanolamine  
and 20% of di-ethanolamine.

30 may proceed as follows: The free fatty acids are combined directly with an organic base or a mixture of such bases. If the fatty acid is a solid the preparation is aided by the application of heat. It is also possible to treat the chloride

The products resulting from this procedure are semi-solids, particularly water soluble and ready for use without further treatment.

35 is also possible to start from the glycerides of the fatty acids, i. e., olive oil, cottonseed oil, castor oil, linseed oil and the like by saponifying the glycerides by heating with the bases to a high temperature. In this case we find

It is possible that the resultant material may be a compound of the base with the oleic acid but this has not been definitely established and is, in fact, immaterial to the success of the invention.

to a high temperature. In this case we find that the reaction is complete when a sample of the mixture dissolves entirely in water. If water is present at the start this may be driven off, the base not being volatile, until a concentrated product is left behind.

The resultant product is a clear yellow oil, very soluble in water.

45 When making these products by this method

The above mixture is heated on the water  $\text{so}$

bath for several hours. The saponification proceeds slowly and in order to make it complete within reasonable time it is of advantage to add an excess, for example 30% tri-ethanolamine, above the quantity mentioned.

*Example 5*

284.39 parts of stearic acid are melted. Into the melt are stirred  
149 parts tri-ethanolamine,—stirring is continued at a temperature of about 80° C. until the mixture is uniform.

10 The resultant product on cooling is a solid, not very soluble in water but very soluble in alcohol. It acts as an excellent assistant in promoting solution.

*Example 6*

282 parts oleic acid  
91 parts of amino-propane diol  
NH<sub>2</sub>—CH<sub>2</sub>—CH—CH<sub>2</sub>—OH  
|  
OH

20 are heated together until completely mixed. The product is very soluble in alcohol. In water the solution is cloudy but becomes clear on the addition of some excess base, e. g. 15 to 20%.

*Example 7*

282 parts oleic acid are caused to react as given in the above example with  
119 parts of methyl di-ethanolamine  
CH<sub>3</sub>—N—(CH<sub>2</sub>—CH<sub>2</sub>OH)<sub>2</sub>.

30 The soap obtained in this way has the property, when in alcoholic solution, of dissolving mercuric oxide and giving a relatively stable product soluble in water. This is altogether a surprising result and illustrates 35 the use of these new soaps for pharmaceutical purposes.

*Example 8*

40 6 parts of a crude sulphonated oil made by the action of sulfuric acid on castor oil are mixed with 1 part of mono-ethanolamine

*Example 9*

2.7 parts of a crude sulphonated oil mixture in the form of free acids are mixed with 1 part of a mixture of di- and tri-ethanolamine.

45 The products of Examples 8 and 9 are entirely soluble in water. They are thick yellow oils presumably containing salts of the bases of the sulfonic acids but this point has not been definitely established and is immaterial to the success of the invention. The 50 products formed in this way are quite satisfactory for ordinary purposes.

In dyeing Ponsol blue GD double paste, Schultz No. 842, on cotton yarn in the package machine, using 5% of color, 2½% sodium hydroxide, 3% hydrosulfite, the addition of 1% of the product formed by combining 1 mole of sulfo-ricinoleic acid and 1 mole tri-ethanolamine, containing di-ethanolamine, results in a brighter, more level dyeing.

60 The use in dying of the new compounds described in this case can be illustrated by the following example:

*Example 10*

65 An 8.5% dyeing of Ponsol blue GD,

Schultz No. 842, on 150 pounds of mercerized cotton piece goods is obtained as follows:

12.75 pounds Ponsol blue GD, Schultz No. 842, are mixed with 8.16 pounds of one of the compounds described in the examples of this case; 1 gallon of cold water is added and the suspension passed through a fine screen. A perfect speckless paste is thus obtained, which is added to the jigger dye bath composed of the following:

10 pounds caustic soda  
15 pounds hydrosulfite concentrated, 10 pounds being added immediately and 5 pounds being added after one passage of the goods  
100 gallons of water.

80 The temperature is raised to 110° F., and after complete reduction the dyeing started at this temperature. The temperature is then allowed to rise during 30 minutes to 125° C., and further dyed at this temperature for 10 to 15 minutes. Then give 1 wash, 4 passages in sodium perborate, 2 lbs. per 100 gals. at 120° F., 2 cold washes, 5 passes in boiling soap solution 3 lbs. soap to 100 gallons, then rinse and wash in the open, dry and calender.

85 This example, illustrating the method of dyeing, is similar to Example 1 given in co-pending application Serial No. 210,715, filed by applicants on August 4, 1927. The 90 difference between this example and the said Example 1 lies in the substitution of the novel assistants herein disclosed by applicants.

*Example 11*

95 The new compounds described in this application may be used as assistants in the making of vat color pastes in a manner similar to the pastes described in applicants' patented application bearing Patent Number 1,705,118, granted March 19, 1929. The 100 dye-stuff paste, as produced in the course of manufacture of Ponsol blue GD, Schultz No. 842, is converted into a press cake containing 30% of dry color. 400 parts of the press cake are then mixed with 20 parts of glycerine 105 and 580 parts of one of the assistants prepared according to Examples 1 to 9 and Example 13 of this application. It is possible to vary the quantities considerably without 110 losing the advantages of this invention.

*Example 12*

115 The new compounds described in this case may be used in printing pastes containing lakes of basic colors. The mode of procedure 120 in using such a printing paste is illustrated in the following example:

125 10 parts basic color (suitable for discharge printing)  
50 parts glycerine  
50 parts of any one of the products described in Examples 1 to 9 and Example 13 of this application  
250 parts water  
580 parts thickening composed of starch or gums and a certain amount of sodium hydrosulfite-formaldehyde necessary to cut the ground  
60 parts tannin dissolved in equal parts of water or alcohol.

The extile or other material printed with this composition is aged and heated, passed into antimony salts, washed, and finished as usual. The process of printing illustrated in this example is identical with Example 4 in applicants' co-pending case Serial No. 195,579, filed May 31, 1927, except for the insertion of the new assistants which comprise part of applicants' herein disclosed invention.

10      *Example 13*

If a pure product is needed the operation may be carried out as follows:

15      378 parts of pure sulfo-ricinoleic acid prepared by the action of chloro-sulfonic acid on pure ricinoleic acid are mixed with 149 parts of tri-ethanolamine.

In the above case the addition of a further molecular equivalent of base produces a more soluble oil. The reason may be that 20 the extra quantity of base combines with the carboxyl group but again this point has not been determined.

In the above examples any one of the bases as defined by the general formula given 25 above may be used either alone or in mixture. The fatty acids may also be varied through a wide range.

By the term "alkyol", as used herein, we mean to include an alkyl radical in which one 30 or more hydrogens are replaced by a hydroxyl group, and may be represented by the following:



35      We have found that these products, which are essentially organic soaps possess a greater dissolving power or dispersing power for organic substances than do ordinary soaps. They possess the detergent property of soaps 40 without the high alkalinity characteristic of sodium or potassium salts of the fatty acids. These products for these reasons have a distinct advantage for many purposes and particularly as assistants in dyeing, and those 45 compounds which are derived from sulfonated castor oil by the process mentioned are in many ways superior to ordinary sulfonated oils. Their superiority is evidenced by the greater evenness of the shades developed, the better utilization of the color, and the greater brillance of the dyeing.

When added to water they bring about solution or dispersion in so fine a form as to appear a solution of insoluble organic bases 55 such as amino-azo-benzene, para-nitro-benzene, azo-diphenylamine, benzene-azo-naphthalene-azo-phenol, Rosanthrene base, diethyl-para-amido-phenol-1:4 naphthoquinone-mono-imide, 2:4 di-nitro-benzene-1:63 azo-di-ethyl-aniline, etc. It takes about 2 to 5 parts of the solvent for 1 part of the insoluble base. These solutions may be used very successfully for the purpose of dyeing fibers of esterified cellulose.

65      It has also been found that these soaps

dissolve metallic hydroxides and oxides, for example, mercuric oxide, and this property indicates their probable value in pharmacology, for example, in the production of anti-septic soaps and the like.

70

As many apparently widely different embodiments of this invention may be made without departing from the spirit thereof, it is to be understood that we do not intend to limit ourselves to the specific embodiments thereof except as indicated in the appended claims.

75      We claim:

1. A printing paste which contains a lake of a basic color and an alkyolamine salt of 80 a higher fatty acid.

2. A printing paste which contains a lake of a basic color and an ethanolamine salt of a higher fatty acid.

3. A printing paste which contains a lake 85 of a basic color and an alkyolamine salt of an acid from the group consisting of oleic, stearic and ricinoleic acids.

4. A printing paste which contains a lake of a basic color and an ethanolamine salt of 90 an acid from the group consisting of oleic, stearic and ricinoleic acids.

5. A printing paste which contains a lake of a basic color and an alkyolamine salt of 95 oleic acid.

6. A printing paste which contains a lake of a basic color and an ethanolamine salt of oleic acid.

7. A printing paste which contains a lake of a basic color and a salt formed by the 100 chemical combination of di-ethanolamine and oleic acid.

8. A printing paste which contains a lake of a basic color and a higher fatty acid salt of a compound having the following formula: 105



110      in which Alk represents an aliphatic or hydroxy aliphatic radical, while both  $\text{R}_1$  and  $\text{R}_2$  represent a monovalent substance from the group consisting of hydrogen, aliphatic radicals, hydroxy aliphatic radicals and polyhydroxy aliphatic radicals.

115

9. A printing paste which contains a lake of a basic color and a compound formed by the chemical combination of an acid from the group consisting of oleic, stearic and ricinoleic acids, together with a compound having the following formula:



120

125      in which Alk represents an aliphatic or hydroxy aliphatic radical, while both  $\text{R}_1$  and  $\text{R}_2$  represent a monovalent substance from the group consisting of hydrogen aliphatic 130

radicals hydroxy aliphatic radicals and polyhydroxy aliphatic radicals.

10. A printing paste which contains a lake of a basic color and a salt formed by the chemical combination of tri-ethanolamine and oleic acid.

11. A printing paste which contains a lake of a basic color and a salt formed by the chemical combination of mono-ethanolamine and oleic acid.

10 In testimony whereof we affix our signatures.

JEAN GEORGES KERN.  
CHARLES J. SALA.

15

20

25

30

35

40

45

50

55

60